

## UNITED STATES PATENT OFFICE

2,324,528

## COPPER-ALUMINUM-MANGANESE ALLOY

Cresap M. Moss, Salt Lake City, Utah, assignor to  
Chicago Development Company, Chicago, Ill.No Drawing. Application August 15, 1941,  
Serial No. 407,904

3 Claims. (Cl. 75—161)

This invention relates to the preparation of certain new and useful alloys of copper, aluminum and manganese and is particularly concerned with such alloys wherein the aluminum content is from about 7% to about 9%, where the manganese content is from approximately 1% to approximately 10%, the balance being substantially all copper, said alloys being essentially entirely free from oxides of aluminum and silicon and containing not more than 0.05% iron.

When manganese is incorporated with aluminum and copper to form an alloy containing up to about 3% manganese, approximately 7.5% aluminum, balance copper, the tensile strength is decreased and the elongation increased over such alloys which are devoid of manganese. With an increase of manganese in such alloys above 4%, the tensile strength increases and the elongation decreases. These properties result when conventional commercial silico-thermic or aluminothermic manganese is utilized in the preparation of the alloys.

In accordance with the present invention, when alloys of the aforementioned type are made from high purity manganese which is essentially free from iron and from the oxides of aluminum and silicon, which impurities are present in commercial silico-thermic and aluminothermic manganese, entirely different results are obtained and the resulting alloys have new and highly improved properties. In order to bring about these results, manganese of a purity of at least 99% should be employed and, for best results, it is especially desirable to utilize electrolytic manganese having a purity of about 99.9%.

In an illustrative example of an alloy made in accordance with the present invention, an alloy was prepared by melting together aluminum, manganese and copper to produce an alloy containing 8% aluminum, 1% manganese, and the balance copper. The metals utilized were all highly pure, the aluminum being Hoopes process aluminum, and the manganese and copper being of the electrolytic variety and having a purity of at least 99.9%. The alloy was cast in a chill mold and hot rolled at 1600 degrees C. The incorporation of the 1% of manganese in the alloy increased the elongation from 20% to 50%, in two inches and, at the same time, the tensile strength was increased from 32,000 pounds per square inch to 48,000 pounds per square inch. Increasing the manganese to 2% of the alloy, while maintaining the aluminum content at about 8%, resulted in decreasing the elongation only slightly, namely, to 46% in two inches, while the tensile strength was increased to 60,000 pounds per square inch.

On sand cast alloys containing about 7.5% aluminum, as much as 6% of high purity manganese may be added without decreasing the

elongation from its original value of 30%, and the tensile strength of such alloys is increased from approximately 20,000 pounds per square inch to 40,000 pounds per square inch. The ability thus greatly to improve both the tensile strength and elongation characteristics of these alloys is of material value.

As indicated hereinabove, the aluminum content of the alloys of the present invention, in its broadest aspects, ranges from about 7% to about 9% and the manganese content ranges from about 1% to about 10%. A particularly preferred range is represented by those alloys which contain from about 7.5% to about 8% of aluminum and from about 1% to about 6% or, better still, from about 1% to 2.5% manganese.

While the best results of the present invention appear to be obtained by utilizing electrolytic manganese of at least 99.9% purity, other forms of substantially pure manganese may also be used such as vacuum distilled manganese and the like. The iron content of the finished alloys should not exceed 0.05% and oxides of aluminum and silicon should be essentially entirely absent.

Those skilled in the art will readily understand the various uses to which the alloys of the present invention may be put in the light of the characteristics and properties which have been described hereinabove.

30. What I claim as new and desire to protect by Letters Patent of the United States is:

1. Alloys of copper, aluminum and manganese containing from about 7 to 9% aluminum, from about 1% to 10% manganese having a purity of at least 99%, balance substantially all copper, said alloys being essentially entirely free from the oxides of aluminum and silicon and containing not more than 0.05% iron.

2. An alloy containing approximately 7.5% aluminum, from about 1% to about 6% manganese having a purity of at least 99%, balance substantially all copper, the alloy being essentially entirely free from the oxides of aluminum and silicon and containing not more than 0.05% iron, said alloy having an elongation in the sand cast condition of at least 30% in two inches and having a tensile strength greater than 20,000 pounds per square inch.

3. An alloy containing approximately 8% electrolytic aluminum, from about 1% to 2.5% electrolytic manganese having a purity of at least 99.9%, balance substantially all electrolytic copper, said alloy being essentially entirely free from the oxides of aluminum and silicon and containing less than 0.05% iron, the alloy having, in the hot rolled condition, an elongation greater than 35% in two inches and a tensile strength greater than 40,000 pounds per square inch.